

July 18, 1933.

R. H. ABORN

1,918,731

WORKING AUSTENITIC STEELS

Filed Feb. 17, 1931

Fig. 1



Fig. 2



Inventor:  
Robert H. Aborn,  
By Uxina & Rauber,  
Attest

## UNITED STATES PATENT OFFICE

ROBERT H. ABORN, OF EAST ORANGE, NEW JERSEY, ASSIGNOR TO UNITED STATES STEEL CORPORATION, OF NEW YORK, N. Y., A CORPORATION OF NEW JERSEY

## WORKING AUSTENITIC STEELS

Application filed February 17, 1931. Serial No. 516,473.

This invention relates to an improved method of treating austenitic metals and is particularly applicable to the working or fabricating of austenitic alloys having corrosion resisting properties.

It has been found that austenitic alloys harden during cold deformation at an unusually rapid rate when the cold work or deformation is applied at, below, and even slightly above, room temperature. The hardening is entirely inordinate and is the cause of the unique properties of the so-called Hadfield manganese austenitic steel. In the instance of the austenitic nickel rustless irons and stainless steels of approximately 18 per cent chromium, 8 per cent nickel and 0.10 per cent carbon the soft recrystallized metal may show a Brinell hardness of 86 and then after working to reduce its thickness by 55 per cent the hardness may reach 400 Brinell, the deformation having been applied at room temperature. On the other hand, non-austenitic metals harden much less, as for example, a very low carbon annealed steel would before work show a Brinell hardness of about 103 and after similar cold work at room temperature develop about 160 Brinell hardness.

The unique property of rapid cold work hardening in the case of austenitic steel is commonly explained by the fact that austenite is not only deformed by the cold work but is also transformed to a different crystalline form, the so-called ferrite or martensitic condition wherein the alpha form of iron is the basis of the crystal, instead of the gamma form, which is the basis in the austenitic metal. At any rate, regardless of the explanation, the transformed metal of austenitic alloys resulting from cold work shows an undesirable brittleness and severe loss of ductility and twist which normal metals do not exhibit. Furthermore, due to the transformation only moderate work is possible before cracks appear unless frequent annealings are employed.

The present invention has for a feature thereof an improved process of cold working austenitic alloys in such a manner that the transformation of austenite to the aforemen-

tioned undesirable modification is very greatly reduced, and in some instances is substantially eliminated. It has been found that this feature can be carried out by cold working (working below the recrystallizing temperature) the austenitic alloys at, or above, about 200 degrees centigrade.

Evidence of the advantages and desirability of the improved process as contrasted with the present day process of cold working the material at, below, or even slightly above room temperature, is afforded by testing the two materials for Brinell hardness and also submitting them to a bend test. Instead of developing about 400 Brinell hardness the alloy treated at or above 250 degrees centigrade shows only about 260 and is vastly more ductile.

In the drawing, Figures 1 and 2 indicate bend tests of material treated first in accordance with the present invention, and second, in accordance with methods now in practice.

As disclosed in Figure 1 of the drawing, a bend test of a small strip showed that the metal worked in accordance with the improved method developed no cracks when bent about a radius less than its own thickness, whereas, the ordinarily worked material broke off before bending about a larger radius.

A quantitative measure of the efficiency of the improved method resides in magnetic measurements which show an entirely different process occurring in the crystalline nature of the metals when worked by the contrasting methods. The same sample of metal worked by the ordinary cold method develops sufficient transformed metal (the non-magnetic form changes to the magnetic form) to produce, for example, 930 magnetic units, while the material worked at 300 degrees centigrade showed only about 10 units. Completely decisive X-ray tests showed correspondingly great differences as to transformation.

It may be remarked incidentally that the energy involved in applying equal deformation to the metal is several times greater at room temperature than at, for example, 300 degrees centigrade.

It is to be appreciated that the term "work-

ing" is used herein in its general sense to include working, fabricating and generally deforming metals. Likewise, it is to be understood that the applicant is to be permitted 5 a certain latitude in respect to the range through which he carries out the improved process. Although for purposes of description the range can perhaps best be defined as below the recrystallizing temperature and 10 above about 200 degrees centigrade, it is pointed out that the treatment contemplated by the invention consists in deliberately or intentionally heating the metal before or during the cold working of it. If the metal is heated 15 during working then to come within the scope of the invention such heating must be deliberate and not as a result of the frictional engagement of the metal and tools. Although it is stated above that for purposes of definition the range can be defined as below the recrystallizing temperature and above about 200 degrees centigrade, it should be explained that working the metal at temperatures as 20 low as 100 degrees centigrade increases substantially the desirable qualities contemplated 25 by the invention.

Having thus described my invention, what I claim as new and desire to secure by Letters Patent of the United States is:

30 1. The method of working austenitic chromium-nickel steels which comprises cold working the same within a temperature range adapted to substantially inhibit allotropic crystal transformation therein, said tempera-

35

ture range being in excess of about 100° C. but below the temperature of recrystallization.

2. The method of working austenitic chromium-nickel steels which comprises cold working the same within a temperature range adapted to substantially inhibit allotropic crystal transformation therein, said temperature range approximating 200° to 400° C. 70

3. The method of working austenitic low carbon chromium, nickel iron alloys which comprises cold working the same within a temperature range adapted to inhibit allotropic crystal transformation, said temperature being in excess of about 100° C. but below the temperature of recrystallization. 75

4. The method of working austenitic steel alloys comprised of about 18% chromium, about 8% nickel, about .10% carbon balance mainly iron, which comprises cold working the same within a temperature range adapted to inhibit allotropic crystal transformation, said temperature range approximating 200° to 400° C. 85

5. As an article of manufacture, a substantially non-magnetic cold worked austenitic chromium-nickel steel alloy. 90

6. As an article of manufacture, a substantially non-magnetic cold worked austenitic steel alloy, said alloy being comprised of about 18% chromium, about 8% nickel, about .10% carbon and balance mainly iron. 95

ROBERT H. ABORN.

100

40

105

45

110

50

115

55

120

60

125

130